

## UNITED STATES PATENT OFFICE

2,056,589

ARTICLES WITH REDUCED TENDENCY  
TO CORRODE

Hermann Schulz and Carl Carius, Dortmund,  
Germany, assignors to the firm Vereinigte  
Stahlwerke Aktiengesellschaft, Dusseldorf,  
Germany

No Drawing. Original application May 31, 1933,  
Serial No. 673,792. Divided and this applica-  
tion June 30, 1936, Serial No. 88,265. In Ger-  
many May 20, 1932

1 Claim. (Cl. 75—125)

The invention relates to articles made from  
steel and cast iron with reduced tendency to cor-  
rode, especially when subjected to the action of  
water, especially sea water and moist soil and  
5 forms a division from our copending application  
Serial No. 673,792, filed May 31, 1933.

The present invention is an improvement of  
the steel and cast iron described and claimed by  
the applicant in his prior application Serial No.  
10 450,878, which matured into Patent No. 2,013,600  
on Sept. 3, 1935, which is also resistant against sea  
water and moist soil. The prior process is based  
upon special electrolytic actions which are there-  
by caused, that the steel or cast iron is alloyed  
15 with copper, antimony, arsenic or tin and in com-  
bination with one or several of these additions  
with magnesium, nickel or aluminum. Said ele-  
ments are used in the prior process in the follow-  
ing amounts: antimony, arsenic, tin in amounts  
20 between 0.05 and 5%, singly or together, copper  
in amounts up to 1%, magnesium between 0.1 and  
5%, aluminum between 0.05 and 5%.

Further researches have shown that the titani-  
um and vanadium elements act in a similar  
25 way as the magnesium and aluminum elements  
used secondly according to the main patent, and  
they are not only equivalent to these elements,  
especially aluminum, but even superior thereto.  
Since this has been found out, it is possible to re-  
30 place the aluminum as well as magnesium partly  
by titanium or vanadium. The favourable influ-  
ence of these two elements could not be foreseen  
either on account of their electrochemical or  
chemical behaviour.

35 A further economically advantageously acting  
influence of titanium and vanadium, owing to  
which steels alloyed with these elements will excel  
compared with aluminum containing steels, is  
that the capacity of steels alloyed with titanium  
40 and vanadium of offering increased resistance to  
the attacks of water will find expression already  
a short time after the beginning of corrosion in  
a considerable reduction of corroding speed. For  
example the corroding speed in sea water will be  
45 reduced already after 14 days approximately 20%  
and in river water about 40% compared with  
that of copper-nickel steels alloyed with alumini-  
num. Steels according to the invention are fur-  
ther distinguished by a perfectly uniform rust-  
50 ing of their surface exposed to the corroding  
agent. Local corrosion attacks in the form of  
dents or holes or notch-like depressions, which  
cause a reduction of the mechanical qualities of  
a steel, do not happen. From the point of view

of foundry technics and metallurgy too, the pos-  
sibility of substituting titanium or vanadium for  
aluminum affords an advantage in so far as steels  
mixed with titanium and vanadium can be worked  
better than those having an addition of alum-  
5 num.

The two elements will have the effect described  
already at very slight amounts thereof, namely,  
if both metals together are present in a quantity  
of 0.1% upwardly, the amount of metals with  
10 respect to their corrosion-stopping influence is  
unlimited. However, it is advisable when adding  
titanium not to exceed 1% and in case of van-  
adium 0.5%, as a greater addition would not afford  
15 any extra advantages.

Thus the invention comprises articles with a  
reduced tendency to corrode under the action of  
a corroding agent, more particularly the moisture  
contained in water, seawater and moist soil; said  
articles being made from a ferrometal alloy con-  
20 taining 0.2-1% copper, titanium between about  
0.1 and 1%, vanadium between about 0.1 and 5%  
and in addition magnesium in amounts between  
about 0.1 and 5% and the balance substantially  
25 all iron, the alloying elements copper, and mag-  
nesium forming together with titanium and vana-  
dium a firmly adhering skin on the articles, due  
to the corroding attack by said corroding agent.

It may be mentioned that the further compo-  
30 sition of the alloys besides the elements above  
specified is the usual one. Thus the alloy may be  
alloyed for some other reasons with the usual  
amounts of elements such as for example man-  
ganese, silicon, phosphorus, chromium, tungsten,  
35 molybdenum, cobalt, boron, zirconium, beryllium,  
as has been stated in my prior patent and in the  
case of steels the accompanying elements may be  
present in approximately the following amounts:

|            | Per cent          |
|------------|-------------------|
| Carbon     | traces up to 1    |
| Silicon    | traces up to 0.5  |
| Manganese  | 0.1 to 1          |
| Sulphur    | traces up to 0.12 |
| Phosphorus | traces up to 0.2  |

40 and in the case of iron in approximately the fol-  
lowing amounts:

|            | Per cent          |
|------------|-------------------|
| Carbon     | 2 to 3.6          |
| Silicon    | 0.3 to 3          |
| Manganese  | 0.3 to 1.2        |
| Sulphur    | traces up to 0.12 |
| Phosphorus | traces up to 1.0  |

55

We claim:

Articles with a reduced tendency to corrode under the action of a corroding agent, more particularly the moisture contained in water, sea-water and moist soil; said articles being made from a ferrometal alloy containing 0.2-1% copper, titanium between about 0.1 and 1%, vanadium between about 0.1 and 0.5% and in addition

magnesium in amounts between about 0.1 and 5% and the balance substantially all iron, the alloying elements copper and magnesium forming together with titanium and vanadium a firmly adhering skin on the articles, due to the corroding attack by said corroding agent. 5

HERMANN SCHULZ.  
CARL CARIUS.